# EUROPEAN PATENT APPLICATION

(11) **EP 1 939 324 A1**
(43) Date of publication of application: **02.07.2008**
(21) Application number: 06077346.2
(22) Date of filing: 29.12.2006
(51) Int. Cl.: C23C 18/30

(54) **Conductive fibrous web and method for making the same**

(71) Applicant: Nederlandse Organisatie voor toegepast-natuurwetenschappelijk Onderzoek TNO, 2628 VK Delft (NL)
(72) Inventor: Kaasjager, Anton, 7523 CH Enschede (NL); Hovestad, Arjan, 5231 PK 's-Hertogenbosch (NL); Jager, Hein, 6723 JB Bome (NL)
(74) Representative: van Loon, C.J.J.

(57) **Abstract**

The invention is directed to a method for making at least part of a fibrous web conductive, to an at least partly conductive fibrous web, and to the use thereof.

The invention seeks to at least partly overcome the disadvantages of electroless plating of a non-conductive surface, such as catalyst penetration through the fibrous web and insufficient spreading of the catalyst on the surface of the fibrous web.

## Description

The invention is directed to a method for making at least part of a non-conductive fibrous web conductive, to an at least partly conductive fibrous web, and to the use thereof.

Conductive fibrous webs, and in particular conductive textiles, are of major interest for applications such as intelligent textiles.

According to the state of the art, non-conductive fibrous webs can be made conductive by weaving a conductive yarn, such as silver yarn, into the web. This allows for instance to make conductive tracks through the fibrous web. Another possibility is to embroider conductive yarn into a non-conductive fibrous web. This allows the creation of certain predetermined conductive patterns. Further methods for making a non-conductive fibrous web conductive include for instance depositing a metal on the fibrous web by physical vapour deposition (PVD) and melting or gluing conductive particles onto the fibrous web.

Disadvantages of the above-mentioned methods include that properties of the fibrous web, such as flexibility , tactile properties and openness, are negatively affected. Further, some of the above-mentioned methods can only be carried out at specific moments in the manufacturing process of the fibrous web. In addition, weaving conductive threads in the web limits the direction of the tracks to the weft and warp direction. The area of the web which can be reached with embroidery is usually limited and depends on the embroidery machine. There is a mismatch between the high cost of silver (in either threads or glued conductive particles) and the low cost fabric. PVD needs to be done under vacuum conditions, which makes it difficult to adopt by the textile industry.

Another possibility for metallising a non-conductive surface is by electroless plating, also known as chemical or autocatalytic plating. This process uses an electrochemical reaction to deposit metal on an object without the passage of an external electric current. Electroless plating involves the deposition of a metal coating onto a substrate by immersing the substrate in a plating solution containing ions of the metal to be deposited and a chemical reducing agent. The metal ions are reduced by the chemical reducing agent in the plating solution, and deposit on the substrate. Metals that can thus be deposited include for instance gold, silver, copper, palladium, nickel, iron, and cobalt.

Parameters which can be controlled in the electroless plating process include the concentration of chemicals, the pH of the plating solution, the amount and type of additives in the plating solution, and the plating temperature.

Electroless plating does not require electrical power. The plating volume and thickness can be controlled and readily varied. Further, electroless plating allows the formation of coatings with uniform thickness, even with irregularly shaped objects.

Metallising a fibrous web by electroless plating is for instance known from US-A-5 599 585. A disadvantage of the method described in US-A-5 599 585 is that by immersing the substrate into the plating solution the entire substrate will be uniformly coated. For certain applications it is desirable to have a conductive pattern on a surface.

WO-A-2005/087979 therefore describes the application of a catalytic activator onto a flat non-fibrous polymer substrate in a pre-selected pattern. The catalytic activator is formed in a two-step procedure by reacting a metal in a positive oxidation state applied in the first step with a reducing agent applied in a second step. According to this publication, the plasma is used to create the catalyst by starting an electrochemical reaction between the metal ion and the reducer that have been separately printed.

The present inventors have now come across the problem that when a catalytic activator is printed on a fibrous web substrate, it penetrates through the fibrous web. This may cause metallisation of both the front and the back of the web during electroless plating. In particular, this problem, which has not been recognised in the prior art, arises when the surface to be treated is a textile fibrous web, such as cotton or polyester fibrous webs.

In a study by Simor et al. (Surf. Coat. Technol. 2003, 172, 1-6) a polyester non-woven fabric was pre-treated with a nitrogen plasma and subsequently metallised with nickel. The catalyst in this study was applied from an aqueous bath. The aim of the plasma in this paper is to obtain a full coverage of the fabric, viz. full coverage of the fibres throughout the fabric. A full coverage of the fabric is important for the object of the study, which is electromagnetic shielding. No distinction is made between the front and the back surface of the fabric. Accordingly, the study is silent with respect to local catalyst adsorption and possible catalyst penetration through the web.

Another problem that the present inventors encountered by using a fibrous web as substrate was that the catalytic activator does not spread sufficiently over the fibres. The fibrous web may therefore lose conductivity when the conductive connection between the different fibres is lost. This is especially problematic when thin conductive tracks are to be applied on the fibrous webs.

Accordingly, an object of the present invention is to at least partly overcome the above-mentioned disadvantages of the prior art. This object has been met by a method in which the substrate is pre-treated with plasma.

Hence, the present invention is directed to a method for making at least part of a fibrous web conductive comprising
- subjecting a surface of the fibrous web to a plasma treatment;
- printing catalyst onto at least part of the plasma treated surface of the fibrous web; and
- metallising at least part of the surface of the fibrous web by immersing the fibrous web in a solution containing metal ions (and a reducing agent).

The method of the invention is simple, quick and allows a control over various parameters. The catalyst is simply applied on the fabric by conventional printing techniques in a one step procedure. The plasma treatment causes chemical activation of the surface, thereby allowing a good spreading of the catalyst over the surface of the fibrous web. At the same time, the plasma treatment activates substantially only one side of the fibrous web and thereby prevents, or at least inhibits, the catalyst from penetrating through the fibrous web. The plasma locally facilitates catalyst adsorption and metal plating. Accordingly, the method of the invention results in a fibrous web which can be metallised uniformly substantially on only one side of the fibrous web.

The inventors found that physical properties of the resulting fibrous web, such as strength, tactile properties and openness are hardly affected by the method of the invention. Furthermore, the process of the invention can be advantageously carried out at atmospheric pressure. The resulting fibrous web has excellent flexibility and may be used for instance in intelligent textiles.

The term "plasma" as used in this application is meant to refer to a partially ionised gas that represents a chemically active environment, which consists of activated species such as electrons, ions, radicals, metastables and photons.

The term "textile" as used in this application is meant to refer to a thin, flexible material made of any combination of cloth, fibre, or polymer.

The term "cloth" as used in this application is meant to refer to a thin, flexible material made from yarns.

The term "yarn" as used in this application is meant to refer to a continuous strand of fibres.

The term "fibre" as used in this application is meant to refer to a unit of matter, either natural, such as cotton, synthetic, such as polyester, or a combination thereof, which forms the basic element of, for example, fabrics, and textile structures. A fibre itself may have a porous structure with voids.

Any type of plasma source may be used. Typical plasma sources include corona discharge, atmospheric pressure glow discharge, microwave discharge, volume filamentary dielectric barrier discharge, volume glow dielectric barrier discharge, plasma jet, micro hollow cathode discharge, surface dielectric barrier discharge, and diffuse coplanar surface barrier discharge. It is preferred that the plasma source is a pulsed plasma source, since this allows a better control over plasma conditions and chemistry.

Preferably, the plasma is applied with a plasma torch involving a plasma jet. This allows for local changes of the wetting behaviour of the surface. The spot size of the plasma and thus the width of the subsequent activated track depend on the design of the plasma torch but can be in the range of millimetres. The fibrous web may be moved underneath the plasma torch or *vice versa.*

The plasma treatment of the surface comprises hydrogen abstraction, radical formation and introduction of new functional groups from the plasma environment. The plasma treatment results in a reactive activated surface.

The spreading behaviour of the catalyst is influenced by the wetting properties of the web. Good wetting properties lead to an excellent spreading over the surface. A high surface energy of the fibres in the web corresponds to good wetting properties. The plasma treatment results in a high surface energy of the fibres in the web. As a result, the catalyst spreads out over the surface of the fibres in the web and thereby minimises the interfacial energy. The plasma treatment is thus a tool to control wetting properties of the surface of the web. Changing the plasma parameters will vary the geometry of the activated surface.

The plasma parameters can be chosen such that the catalyst is selectively attached to a first side of the fibrous web, or at least more than readily than to a second side of the fibrous web. The second side of the web can be metallised separately, for instance with a different metal or mixture of metals.

The application of two different conductive coatings on both sides of the fibrous web may be improved by applying a separating coating. This coating can applied on the second side of the web, before or after the first side has been metallised. The coating may be a conventional coating and is for instance applied by a blade or a knife. The following materials can be used for these coatings: silicones, acrylates, polyurethanes, co-polymers, ethylene phenyl acetate, sol gel coatings and plasma deposited coatings. Preferably, the coating is a very thin coating, for example less than 100 nm, more preferably less than 5-50 nm. The coating and the plasma parameters can be tuned so that the wetting properties of the second side of the fibrous web when applying the second metal layer are such that the metal is selectively attached to the second side of the fibrous web, or at least more than readily than to the first side of the fibrous web.

According to the method of the invention, catalyst is printed onto the surface of the fibrous web. This may be done after the surface of the fibrous web has been subjected to the plasma treatment. This allows the production of a fibrous web with a pre-designed conductive pattern.

In case no specific conductive pattern is required, the catalyst can also be printed simultaneously with the plasma treatment. This is advantageous because the total amount of production steps is reduced.

The catalyst can be printed onto the surface of the fibrous web by conventional printing techniques, such as screen printing, valve jet printing and inkjet printing. Preferably, the catalyst is printed by valve jet printing or inkjet printing.

Screen printing involves a costly mask, the screen, which is absent in inkjet printing and the use of a valve jet. This makes the latter two techniques more flexible. It also means that there is no need for a repetitive design in the case of inkjet or valve jet printing. Computer Aided Manufacturing is easy to implement.

Screen printing is done with pastes with a relatively high viscosity. The wetting of the fabric by these pastes will be more controlled by the viscosity than by the wetting properties of the surface of the fabric. The pastes with relatively high viscosity require specialised catalyst formulations that are more expensive and less effective. In inkjet printing standard catalyst formulations without modification can be used.

With a valve jet a larger amount of liquid is added to the substrate due to a bigger drop size, typically about 1 g of liquid on 1 g of fabric. With inkjet this relation is 10 to 100 times smaller, so 0.1 to 0.01 g liquid on 1 g of fabric. The amount applied by both jet techniques is so small that wetting of the fabric can be controlled locally. Valve jet results in a higher production speed, because more liquid can be applied but needs better control of the wetting of the surface.

In an embodiment of the invention, the printing technique is incorporated in the plasma. For example, the printing technique, preferably a valve jet or an inkjet, can be incorporated in a plasma torch.

Any catalyst may be used that is able to catalyse the reduction of the metal to be deposited in the electroless plating step. Examples of such catalysts include palladium, gold, silver, copper, tin, nickel, cobalt, iron, aluminium, zinc, molybdenum, tungsten, niobium, titanium, tantalum, ruthenium, and platinum.

Only a very small amount of catalyst is required. Typically, an amount of 0.1-100 mg/m², preferably 5-50 mg/m², for instance 10 mg/m² of catalyst is printed on the fibrous web.

According to the invention, the plasma treated surface of the fibrous web with catalyst is then immersed in a plating solution which comprises metal ions and a reducing agent. The plating solution is typically an aqueous solution. The reducing agent reduces the metal ions which deposit on the surface when the oxidation number has reached zero. This metallising technique is known as electroless plating. The catalyst on the surface of the fibrous web catalyses the electrochemical reaction and therefore, the metal will deposit on the areas of the surface where catalyst is printed. This allows to create specific metallised patterns on the surface of the fibrous web.

Suitable metal ions for obtaining a conductive fibrous web are for example gold ions, silver ions, copper ions, nickel ions, tin ions, platinum ions, cobalt ions, palladium ions, iron ions and lead ions. It is also possible to apply a mixture of metal ions and then obtain a fibrous web with an alloy coating. Preferred metal ions are gold ions and copper ions. Normally the metal ions are provided in the solution by dissolving a metal salt.

Typical electroless copper baths can be divided into two types: heavy deposition baths (designed to produce 2 to 5 µm of copper) and light deposition baths (designed to produce 0.50 to 1.00 µm of copper). The main constituents of typical electroless copper chemistry are sodium hydroxide, a reducing agent such as formaldehyde, ethylenediaminetetraacetic acid (EDTA) or another chelator, and a copper salt. In the complex reaction, which may be catalysed by palladium, the reducing agent reduces the copper ion to metallic copper. Formaldehyde (which is oxidised), sodium hydroxide (which is consumed), and copper (which is deposited) must be replenished frequently.

The reducing agent used in the plating solution is preferably a mild reducing agent, such as formaldehyde, a formiate, dimethylaminoborane, diethylaminoborane, hydrazine, hypophosphite, or boron hydride.

The concentration of metal ions in the plating solution is in general 1-10 g/l. The concentration of the reducing agent is typically 1-50 ml/l. The ratio between the metal ions concentration and the reducing agent concentration can range from 0.1 to 2, preferably from 0.3 to 1.

It is advantageous to stretch the fibrous web during the printing of the catalyst and during the metallising of the fibrous web. This facilitates the deposition process and increases the robustness of the resulting at least partly conductive fibrous web. Furthermore, the density of the conductive fibres in the fibrous web after relaxation is higher than the density of the conductive fibres when the deposition took place onto a non-stretched fibrous web.

The fibrous web can be a knitted or woven textile or a non-woven. Preferably, the fibrous web is a textile made from any combination of materials normally used in textiles, such as polyester, cotton, polyamide, polyacryl, wool, and silk.

In a further embodiment of the invention, both front and back surface of the fibrous web are metallised with a different metal or mixture of metals. Since the invention allows to selectively metallise a certain surface of the fibrous web, it is possible to provide both front and back surface of the fibrous web with a different metal coating.

The invention is further directed to an at least partly conductive fibrous web which is obtainable by the inventive method. It has been found that the conductive metal coatings that are applied by the method of the invention are improved over the prior art metal coatings. The connection between the different metallised fibres is better, because the catalyst spreads better over the fibres. Furthermore, the catalyst does not penetrate through the fibrous web. Hence, a fibrous web can be obtained which has a pre-selected conductive surface, while the opposite surface is not, or at least much less, conductive.

The at least partly conductive fibrous web of the invention can be used as a base to produce all kinds of devices on a fibrous web, including antennas, transmitters, solar cell, batteries, sensors etc.

Advantageously, the at least partly conductive fibrous web of the invention is used for instance in intelligent textiles. The conductivity of the fibrous web is the result of the contact of different fibres in the fibrous web. The conductivity of such a structure changes upon stretching. This effect can be used to use the at least partly conductive fibrous web of the invention as an inductive or deformation sensor. Particularly interesting are the detection and monitoring of body activity, such as breathing, heart beat, posture and movement. For this use the at least partly conductive fibrous webs of the invention can be used as clothing, bedclothes etc.

Furthermore, conductive fibrous webs may be used for the integration of communication apparatuses (such as cell phones) and entertainment apparatuses (such as MP3 players) in clothing. In this regard, the conductive metallic pattern can be used as an antenna, or wiring for receiving signals, or for the provision of power to a connected device.

The at least partly conductive fibrous web of the invention can also be used for manufacturing electrically heatable fibrous webs, such as bed sheets, blankets, furnishing fabrics and for clothing.

As used in clothing or bedclothes, the invention is especially applicable in sportswear and in medical appliances, both for acting as sensor or to apply heat to the body.

## Claims

1. Method for making at least part of a fibrous web conductive comprising
- subjecting a surface of the fibrous web to a plasma treatment;
- printing catalyst onto the surface of the fibrous web; and
- metallising at least part of the surface of the plasma treated fibrous web with catalyst by immersing the surface of the fibrous web in a plating solution which comprises metal ions and a reducing agent.

2. Method according to claim 1, wherein the catalyst is printed after the plasma treatment of the surface of the fibrous web.

3. Method according to claim 1, wherein the catalyst is printed simultaneously with the plasma treatment.

4. Method according to any one of claims 1-3, wherein the catalyst is printed by a method selected from the group of valve jet printing and inkjet printing.

5. Method according to any one of claims 1-4, wherein the catalyst is selected from the group consisting of palladium, gold, silver, copper, tin, nickel, cobalt, iron, aluminium, zinc, molybdenum, tungsten, niobium, titanium, tantalum, ruthenium, platinum, and mixtures thereof.

6. Method according to any one of claims 1-5, wherein the metal ions are selected from the group consisting of gold ions, silver ions, copper ions, nickel ions, tin ions, platinum ions, cobalt ions, palladium ions, iron ions and lead ions, and mixtures thereof.

7. Method according to any one of claims 1-6, wherein the reducing agent is selected from the group consisting of formaldehyde, a formiate, dimethylaminoborane, diethylaminoborane, hydrazine, hypophosphite, and boronhydride.

8. Method according to any one of claims 1-7, wherein the plasma treatment comprises subjecting the surface of the fibrous web to a plasma torch.

9. Method according to any one of claims 1-8, wherein the fibrous web is selected from the group consisting of a textile, a polymer web, a nanofibre non-woven, and a felt.

10. Method according to any one of claims 1-9, wherein the fibrous web is a textile comprising at least one material selected from the group consisting of polyester, cotton, polyamide, polyacryl, wool, and silk.

11. Method according to any one of claims 1-10, wherein the front and back surface of the fibrous web are metallised with a different metal or different mixture of metals.

12. An at least partly conductive fibrous web obtainable by a method according to any one of claims 1-11.

13. Use of an at least partly conductive fibrous web according to claim 12 as a deformation sensor or an inductive sensor.

14. Use of an at least partly conductive fibrous web according to claim 12 for heating.

15. Use of an at least partly conductive fibrous web according to claim 12 as an antenna or wiring for a device.

16. Bedclothes comprising an at least partly conductive fibrous web according to claim 12.

17. Sportswear comprising an at least partly conductive fibrous web according to claim 12.

18. Medical appliance comprising an at least partly conductive fibrous web according to claim 12.
